

# UNITED STATES PATENT OFFICE.

EMILE BRONNERT, OF MULHAUSEN, FRANCE.

## MANUFACTURE OF ARTIFICIAL SILK.

1,387,882.

Specification of Letters Patent. Patented Aug. 16, 1921.

No Drawing.

Application filed September 2, 1920. Serial No. 407,753.

To all whom it may concern:

Be it known that I, EMILE BRONNERT, a citizen of the Republic of France, residing at 1 Quai du Barrage, Mulhausen, Alsace 5 Lorraine, France, have invented certain new and useful Improvements in or Relating to the Manufacture of Artificial Silk, for which I have filed applications in Germany, May 19, 1919; France, Apr. 7, 1920; Netherlands, Apr. 7, 1920; Italy, Apr. 7, 1920; Austria, Apr. 7, 1920; Switzerland, filed Apr. 7, 1920; Belgium and England, filed May 7, 1920,) of which the following is a specification.

15 It is well known that in the production of artificial silk threads from raw viscose by means of mineral acids, very fresh viscose, can be spun even with pure sulfuric acid, provided that the action of the acid 20 is not too violent.

Instead of adding sulfates in such quantities that the ionization of the acids is rendered ineffective (that is beyond the bisulfate proportion or an acid concentration 25 of about 20%), it is preferable to use a relatively weak acid (about 10% concentration), while the decomposing power is further restricted by the briefness of the action of the acid, so that even at somewhat increased temperature of the latter, it can 30 have no appreciable bad influence on the thread. The strong cooling taking place during the emergence of the thread from the bath and the comparatively long distance it 35 has to travel to the receiving member, is very advantageous.

Now, I have found that with sulfuric acid alone (at a temperature of about 45° Celsius), and with the usual spinning length of 40 150 mm., a soft full-bodied thread can be obtained with great certainty, even with viscose of widely different ages, provided sulfuric acid be used which is wholly or partially bound to aromatic radicals.

45 My invention is illustrated by the following examples.

### Example 1.

The spinning bath consists of a solution 50 of 100 gr. sodium benzenesulfonate and 120 gr. sulfuric acid monohydrate per liter. This solution can be used at a temperature of 45° for spinning raw viscose of the usual composition through the usual nozzles of 55 0.10 mm. diameter by calculating the feed of spinning solution corresponding to a

drawing speed of 45 m. per minute and the number of nozzle apertures to an individual thread strength of about 7 deniers.

With ripenesses of 6° (chlorid of ammonium standard) up to ripenesses of about 9°, there are obtained perfectly fine, soft, full-bodied, highly lustrous threads of good tenacity and elasticity.

With fresher viscose, however, of about 12° ripeness not a highly lustrous, but only a matt or dull thread is obtained, but, nevertheless, not the lusterless cotton-like product which is otherwise occasionally obtained when the degree of ripeness of the viscose 70 and the degree of acidity of the bath are not brought into proper relation.

### Example 2.

The spinning bath consists of a solution 75 of 200 gr. sodium benzenesulfonate and 120 gr. sulfuric acid mono-hydrate.

The spinning conditions are observed as in Example 1.

This time, with ripenesses of about 6° to 80 12°, excellent, soft, full-bodied threads are obtained.

It was observed that riper viscose has the tendency to yield a somewhat firmer but somewhat less elastic or stretchable silk, 85 while fresher viscose gives a somewhat less firm, but hence all the more elastic thread, for instance in the present case up to 18% and more.

By varying the degree of ripeness it is 90 therefore possible to regulate the expansibility of the threads which is so essential for weaving purposes.

Instead of sodium benzenesulfonate there can also be used the direct sulfonation mixture of the benzene or of its homologues, its oxy- or other derivatives, or of the condensation products thereof, and when I speak on my claims of sodium benzenesulfonate, I mean to include the above mentioned homologues, condensation products or derivatives.

Owing to the fact that it is generally unnecessary to make a separation of the various isomers formed, and that the tedious transmutation into sodium salt is not necessary, the process appears to be especially economical.

The process can be used for silk of the ordinary size or for very fine threads. For the latter the concentration of the free acid 110 must be in the well known relation to the titre of the threads.

What I claim is:

1. The process of making artificial viscose silk, which comprises treating viscose in a precipitating bath comprising a solution of sodium benzenesulfonate and sulfuric acid monohydrate.
2. A bath for treating viscose, comprising 200 grams or less of sodium benzenesulfonate per liter.
3. A bath for treating viscose, comprising 100 grams of sodium benzenesulfonate per liter.
4. A bath for treating viscose, comprising sodium benzenesulfonate.
5. A bath for treating viscose, comprising 15 a sulfonation product of benzene or its homologues.

In witness whereof, I have hereunto signed my name in the presence of two subscribing witnesses.

EMILE BRONNERT.

Witnesses:

L. R. SE JALIS,  
N. SCHLUMBORGE.